



US005141145A

**United States Patent** [19]

Das et al.

[11] **Patent Number:** **5,141,145**[45] **Date of Patent:** **Aug. 25, 1992**

[54] **ARC SPRAYED CONTINUOUSLY REINFORCED ALUMINUM BASE COMPOSITES**

[75] Inventors: **Santosh K. Das; Michael S. Zedalis, both of Randolph, N.J.; Paul S. Gilman, Suffern, N.Y.**

[73] Assignee: **Allied-Signal Inc., Morris Township, Morris County, N.J.**

[21] Appl. No.: **435,149**

[22] Filed: **Nov. 13, 1989**

**Related U.S. Application Data**

[63] Continuation-in-part of Ser. No. 435,136, Nov. 9, 1989, abandoned.

[51] Int. Cl.<sup>5</sup> ..... **B23K 20/00; B23K 103/16**

[52] U.S. Cl. ..... **228/121; 228/120; 228/175; 228/190; 228/194; 228/243; 164/477; 164/76.1**

[58] **Field of Search** ..... **228/190, 120, 175, 243, 228/193, 194, 121, 122, 124, 263.12, 263.17; 427/423, 34; 164/46, 97, 477, 76.1; 148/403**

[56]

**References Cited****U.S. PATENT DOCUMENTS**

|           |         |                        |            |
|-----------|---------|------------------------|------------|
| 3,609,855 | 10/1971 | Schmidt .....          | 228/190    |
| 3,795,042 | 5/1974  | Kreider et al. ....    | 228/190    |
| 3,900,150 | 8/1975  | Delgrossio et al. .... | 228/190    |
| 4,010,884 | 3/1977  | Rothman .....          | 228/190    |
| 4,298,382 | 11/1981 | Stempin et al. ....    | 228/190    |
| 4,518,625 | 5/1985  | Westfall .....         | 219/76.14  |
| 4,529,457 | 7/1985  | Kushnick .....         | 228/190    |
| 4,529,458 | 7/1985  | Kushnick et al. ....   | 228/190    |
| 4,786,566 | 11/1988 | Siemers .....          | 228/263.12 |
| 4,847,044 | 7/1989  | Ghosh .....            | 228/263.17 |

*Primary Examiner*—Sam Heinrich

*Attorney, Agent, or Firm*—Ernest D. Buff; Gerhard H. Fuchs

[57]

**ABSTRACT**

A metal matrix composite is produced by forming a rapidly solidified aluminum base alloy into wire. The wire is arc sprayed onto at least one substrate having thereon a fiber reinforcing material to form a plurality of preforms. Each of the preforms has a layer of the alloy deposited thereon, and the fiber reinforcing material is present in an amount ranging from about 0.1 to 75 percent by volume thereof. The preforms are bonded together to form an engineering shape.

**25 Claims, 2 Drawing Sheets**



Fig. 1



Fig. 2



Fig. 3



## ARC SPRAYED CONTINUOUSLY REINFORCED ALUMINUM BASE COMPOSITES

### CROSS HEADINGS FOR RELATED APPLICATIONS

This application is a continuation-in-part of application Ser. No. 07/435,136, filed Nov. 9, 1989 now abandoned.

### BACKGROUND OF THE INVENTION

#### 1. Field of the Invention

This invention relates to a process for improving the mechanical properties of metals, and more particularly to a process for producing an aluminum composite having a rapidly solidified metal matrix and a continuous fiber reinforcement.

#### 2. Description of the Prior ART

An aluminum based composite generally comprises two components—an aluminum alloy matrix and a hard reinforcing second phase. The reinforcing Phase may be discontinuous, e.g., particulate, short fiber, or may be continuous in the form of a fiber or tape. The composite typically exhibits at least one characteristic reflective of each component. For example, a continuous fiber reinforced aluminum based composite should reflect the ductility and fracture toughness of the aluminum matrix as well as the elastic modulus and strength of the fiber.

Continuous fiber reinforced aluminum based composites are usually limited to ambient temperature applications because of the large mismatch in higher temperature strength between the aluminum matrix (low strength) and the continuous fiber reinforcement (high strength). Another problem with continuous fiber reinforced metal matrix composites produced by mechanically binding continuous fiber between aluminum based matrix foils is the difficulty in producing a bond between the matrix and the fiber. To produce such a bond it is often times necessary to vacuum hot press the material at temperatures higher than the incipient melting temperature of the matrix or higher than the stability of dispersed phases present in the aluminum based matrix. Still another problem with continuous fiber reinforced metal matrix composites produced by cold spraying a rapidly solidified aluminum based matrix mixed with an organic binder onto a continuous fiber preform and then burning off the organic binder is that the organic binder decomposes and forms a deleterious residue within the sprayed preform. An alternative method of fabricating the composites is by arc spraying. Prior processes in which alloys and/or continuous fiber reinforced metal matrix composites are fabricated by means of arc spraying is disclosed in U.S. Pat. No. 4,518,625. However, the previous work was done using atomized aluminum powder which did not have the metastable microstructure of rapidly solidified aluminum powder. Hence, there is a need for an invention for arc spraying a rapidly solidified aluminum alloy matrix where rapid enough solidification of the molten powder droplets be attained to retain the microstructure of the starting rapidly solidified alloy.

### SUMMARY OF THE INVENTION

It is therefore proposed that the elevated temperature properties of the composite be improved, and these two latter techniques for fabrication be avoided by arc spraying a rapidly solidified, high temperature aluminum alloy onto continuous fiber preforms. This proce-

dure, referred to as arc spraying, provides for a high temperature aluminum base matrix free of organic residue and permits the continuous fiber reinforcement to be bonded to the matrix without heating the material to a temperature above the solidus of the matrix. Moreover, this procedure allows for the deposition and retention of a rapidly solidified alloy onto a substrate and the improved ambient and elevated temperature mechanical and physical properties accorded from the resultant microstructure. The arc sprayed monotapes may be subsequently bonded together using suitable bonding techniques, e.g., diffusion or roll bonding, forming engineering structural components.

Briefly stated, the invention provides a process for producing a rapidly solidified aluminum base metal matrix composite, comprising the steps of: (a) forming a rapidly solidified aluminum base alloy into a wire; (b) arc spraying said wire onto at least one substrate having thereon a fiber reinforcing material to form a plurality of preforms wherein each of said preforms has a layer of said alloy deposited thereon and said fiber reinforcing material is present in an amount ranging from about 0.1 to 75 percent by volume thereof; and (c) bonding said preforms to form an engineering shape.

In addition, the invention provides a composite comprised of a plurality of preforms bonded to form an engineering shape, each of said preforms comprising a substrate having thereon a fiber reinforcing material upon which an aluminum base alloy layer is deposited, said alloy having been rapidly solidified, formed into a wire and deposited by arc spraying, and said fiber reinforcing material being present in an amount ranging from about 0.1 to 75 percent by volume thereof.

Wire having a diameter suitable for arc spraying may be fabricated directly by a friction actuated process or by conventional wire drawing techniques, and sprayed onto a fiber reinforced substrate using arc spraying techniques to form preform monotapes. The fiber may be placed directly on a mandrel or on a suitable substrate such as a rolled foil or planar flow cast ribbon, and is present in an amount ranging from about 0.1 to 75 percent by volume of the sprayed monotape. In this manner there is provided a strong bond between the deposited matrix material and the surface of the reinforcing fibers. Moreover, the attractive microstructure and mechanical and physical properties of the rapidly solidified wire are retained. This process may be repeated such that subsequent spraying is done on fibers placed on top of the sprayed monotapes, and the multi-layered preforms may be fabricated. Upon completion of the arc spraying step, the resultant fiber reinforced preforms are bonded together using suitable bonding techniques such as diffusion bonding, roll bonding and/or hot isostatic pressing, to form an engineering shape which is substantially void-free mass. This shape may be subsequently worked to increase its density and provide engineering shapes suitable for use in aerospace components such as stators, wing skins, missile fins, actuator casings, electronic housings and other elevated temperature stiffness and strength critical parts, automotive components such as piston heads, piston liners, valve seats and stems, connecting rods, cank shafts, brake shoes and liners, tank tracks, torpedo housings, radar antennae, radar dishes, space structures, sabot casings, tennis racquets, golf club shafts and the like.

## BRIEF DESCRIPTION OF THE DRAWINGS

This invention will be more fully understood and further advantages will become apparent when reference is made to the following detailed description of the preferred embodiment of the invention and the accompanying drawings in which:

FIG. 1 is a light photomicrograph of fiber reinforced arc sprayed monotapes composed of rapidly solidified aluminum based iron, vanadium and silicon containing alloy matrix deposited on reinforced British Petroleum Sigma monofilament SiC fiber placed upon planar flow cast aluminum based iron, vanadium and silicon containing ribbon fabricated by the present invention;

FIG. 2 is a light photomicrograph of fiber reinforced arc sprayed monotapes composed of rapidly solidified aluminum based iron, vanadium and silicon containing alloy matrix deposited on Nicalon multi-filament SiC fiber impregnated with aluminum, placed upon planar flow cast aluminum based iron, vanadium and silicon containing ribbon fabricated by the present invention;

FIG. 3 is a transmission electron photomicrograph of a deposited layer of arc sprayed alloy composed of rapidly solidified aluminum based iron, vanadium and silicon containing alloy fabricated by the present invention;

## DESCRIPTION OF THE PREFERRED EMBODIMENTS

The aluminum base, rapidly solidified alloy appointed for use in the process of the present invention has a composition consisting essentially of the formula  $Al_{ba}Fe_aSi_bX_c$  wherein X is at least one element selected from the group consisting of Mn, V, Cr, Mo, W, Nb, Ta, "a" ranges from 1.5-8.5 at %, "b" ranges from 0.25-5.5 at %, "c" ranges from 0.05-4.25 at % and the balance is aluminum plus incidental impurities, with the proviso that the ratio  $[Fe+X]:Si$  ranges from about 2.0:1 to 5.0:1. Examples of the alloy include aluminum-iron-vanadium-silicon compositions wherein the iron ranges from about 1.5-8.5 at %, vanadium ranges from about 0.25-4.25 at %, and silicon ranges from about 0.5-5.5 at %.

Another aluminum base, rapidly solidified alloy suitable for use in the process of the invention has a composition consisting essentially of the formula  $Al_{ba}Fe_aSi_bX_c$  wherein X is at least one element selected from the group consisting of Mn, V, Cr, Mo, W, Nb, Ta, "a" ranges from 1.5-7.5 at %, "b" ranges from 0.75-9.5 at %, "c" ranges from 0.25-4.5 at % and the balance is aluminum plus incidental impurities, with the proviso that the ratio  $[Fe+X]:Si$  ranges from about 2.0:1 to 1.0:1.

Still another aluminum base, rapidly solidified alloy suitable for use in the process of the invention has a composition consisting essentially of the formula  $Al_{ba}Fe_aX_c$  wherein X is at least one element selected from the group consisting of Mn, V, Cr, Mo, W, Nb, Ta, Ce, Ni, Zr, Hf, Ti, Sc, "a" ranges from 1.5-8.5 at %, "b" ranges from 0.25-7.0 at %, and the balance is aluminum plus incidental impurities.

Still another aluminum base, rapidly solidified alloy that is suitable for use in the process of the invention has a composition range consisting essentially of about 2-15 at % from the group consisting of zirconium, hafnium, titanium, vanadium, niobium, tantalum, erbium, about 0-5 at % calcium, about 0-5 at % germanium, about 0-2

at % boron, the balance being aluminum plus incidental impurities.

A low density aluminum-lithium base, rapidly solidified alloy suitable for use in the present process has a composition consisting essentially of the formula  $Al_{ba}Zr_aLi_bMg_cT_d$ , wherein T is at least one element selected from the group consisting of Cu, Si, Sc, Ti, B, Hf, Cr, Mn, Fe, Co and Ni, "a" ranges from 0.05-0.75 at %, "b" ranges from 9.0-17.75 at %, "c" ranges from 0.45-8.5 at % and "d" ranges from about 0.05-13 at %, the balance being aluminum plus incidental impurities.

Those skilled in the art will also appreciate that other dispersion strengthened, rapidly solidified alloys may be appointed for use in the process of the present invention.

The metal alloy quenching techniques used to fabricate these alloys generally comprise the step of cooling a melt of the desired composition at a rate of at least about 10<sup>5</sup> °C./sec. Generally, a particular composition is selected, powders or granules of the requisite elements in the desired portions are melted and homogenized, and the molten alloy is rapidly quenched on a chill surface, such as a rapidly moving metal substrate, an impinging gas or liquid.

When processed by these rapid solidification methods the aluminum alloy is manifest as a ribbon, powder or splat of substantially uniform microstructure and chemical composition. The substantially uniformly structured ribbon, powder or splat may then be pulverized to a particulate for further processing.

By following this processing route to manufacture the aluminum matrix, the rapidly solidified aluminum alloy particulate has properties that make it amenable to direct friction actuated extrusion into wire, as well as numerous powder metallurgy techniques used to fabricate such powders include vacuum hot degassing and compacting the rapidly solidified powder into near fully dense billets at temperatures where the majority of the absorbed gases are driven from the powder surfaces and that decomposition of any dispersed phases does not occur. The billets may thereafter be compacted to full density in a blind die extrusion press, forged, or directly extruded into various shapes including profiled extrusions and wire.

For the purposes of this specification and claims the term fiber means a ceramic material continuous in length and not of a prescribed diameter or chemical composition. Moreover, the term reinforcement of the composite shall mean (1) an essentially nonmalleable character, (2) a scratch hardness in excess of 8 on the Ridgway's Extension of the MOHS' Scale of Hardness and (3) an elastic modulus greater than 200 GPa. However, for the aluminum matrices of this invention somewhat softer reinforcing fibers such as graphite fibers may be useful. Reinforcing fibers useful in the process of this invention include mono- and multi-filaments of silicon carbide, aluminum oxide including single crystal sapphire and/or aluminum hydroxide (including additions thereof due to its formation on the surface of the aluminum matrix material), zirconia, garnet, cerium oxide, yttria, aluminum silicate, including those silicates modified with fluoride and hydroxide ions, silicon nitride, boron nitride, boron carbide, simple mixed carbides, borides carbo-borides and carbonitrides of tantalum, tungsten, zirconium, hafnium and titanium, and any of the aforementioned fibers impregnated or encompassed with a metal such as aluminum, titanium, copper, nickel, iron or magnesium. In particular, be-

cause the present invention is concerned with aluminum based composites that possess a relatively low density and high modulus, silicon carbide and aluminum oxide are desirable as the reinforcing phase. However, depending on the rapidly solidified alloy other fiber reinforcements may prove to form superior matrix/reinforcement bonds. Also, the present specification is not limited to single types of reinforcement or single phase matrix alloys.

In the process of the present invention fibers are initially placed directly on a mandrel or on a suitable substrate such as a rolled foil or planar flow cast ribbon in an amount ranging from about 0.1 to 75 percent by volume of the sprayed monotape. The mandrel may be water or gas cooled, or may be heated directly or indirectly during the processing. The optimum mandrel temperature is dependent on the rapidly solidified alloy and the dispersed phases which must be formed during solidification. The rapidly solidified alloy in the form of a wire is arc sprayed to form a preform such as a monotape.

The arc spraying step comprises the steps of (i) striking an arc between two strands of said wire to melt the tips thereof; and (ii) atomizing said melt in said arc by impinging a high pressure inert gas thereagainst. Specifically, arc spraying involves initially striking an arc between two strands of a conductive metal wire and essentially atomizing any molten metal which forms in the arc by impinging a high pressure inert gas onto the molten wire tips. Since arc spraying is a consumable process, wire is continually fed and the arc and metal source are maintained. The rapidly solidified alloy must be provided as a wire that can range in size from 0.05 cm to 0.25 cm in diameter and more preferably from about 0.1 cm to 0.18 cm in diameter, the optimum wire diameter depending on the alloy composition, the voltage across the wires and the feed sizes physically allowed by the arc spraying apparatus. The wire suitable in diameter for arc spraying may be fabricated directly by a friction actuated process or by conventional wire drawing techniques.

Arc spraying may be performed for varying lengths of time depending on the thickness of the sprayed preform required. In this manner there is provided a strong bond between the deposited matrix material and the surface of the reinforcing fibers. Moreover, the attractive microstructure and mechanical and physical properties of the rapidly solidified wire are retained. This process may be repeated such that subsequent spraying is done on fibers placed on top of the sprayed monotapes, and multi-layered preforms may be fabricated. That is to say, additional fiber reinforcing material can be applied to each of said preforms and said wire arc sprayed thereon to modify said preforms prior to bonding.

The fabricated fiber reinforced preforms may be bonded together using suitable bonding techniques such as diffusion bonding, roll bonding and/or hot isostatic pressing, to form an engineering shape which is a substantially void-free mass. Bonding may be performed at temperatures which range from 400° C. to 575° C. and more preferably in the range from 475° C. to 530° C., under applied pressures which range from 7 MPa to 150 MPa and more preferably in the range from 34 MPa to 100 MPa. The applied pressure is dependent on the bonding temperature and optimally will be sufficient to provide a mechanical and chemical bond between preforms, yet will not break or damage the fibers present in

the preform. In the case of diffusion bonding or hot isostatic pressing, vacuums greater than 100 microns are preferable. Bonding may be assisted by placing foils or powders composed of commercially pure aluminum or of a suitable alloy which is relatively soft at the bonding temperatures and allows fast diffusion of alloy constituents across the foil/preform boundaries. Moreover, fiber reinforced preforms may be oriented above one another such that the fiber reinforcement may be unidirectional, bi-directional or multi-directional. The number of laminations is dependent on the required size and thickness of the desired engineering shape. This shape may be subsequently worked to increase its density and provide engineering shapes such as sheets and plates suitable for use in aerospace, automotive and miscellaneous components.

#### EXAMPLE I

Rapidly solidified, planar flow cast ribbon of the composition aluminum balance, 4.06 at % iron, 0.70 at % vanadium, 1.51 at % silicon (hereinafter designated alloy A) was wrapped on about a 30 cm diameter steel mandrel. British Petroleum Sigma monofilament SiC fiber (hereinafter designated BP fiber) was then wrapped on top of the planar flow cast substrate. The BP fiber has an average diameter of about 104 micrometers and were wrapped with about a 300 micrometer spacing. 16 gauge (approximately 0.16 cm diameter) wire composed of alloy A was then arc sprayed onto the BP fiber wrapped mandrels for approximately 0.5 min. Arc spraying was performed at approximately 34 volts, 100 amps to deposit the required layer of rapidly solidified alloy A. FIG. 1 is a light photomicrograph of fiber reinforced arc sprayed monotape composed of rapidly solidified aluminum base alloy A deposited on reinforced BP placed upon planar flow cast aluminum based alloy A ribbon fabricated by the present invention. Some porosity may be observed due to the fact that arc spraying is not done in vacuum, however, discrete primary intermetallic compound particles are not seen in the matrix alloy A microstructure indicating that solidification of the arc sprayed metal droplets occurs at a rate rapid enough to suppress the formation of coarse primary dispersoid particles.

#### EXAMPLE II

Rapidly solidified, planar flow cast ribbon of the composition aluminum balance, 4.06 at % iron, 0.70 at % vanadium, 1.51 at % silicon (hereinafter designated alloy A) was wrapped on about a 30 cm diameter steel mandrel Nicalon multifilament SiC fiber impregnated with aluminum (hereinafter designated Nicalon fiber) was then wrapped on top of the planar flow cast substrate. The Nicalon fiber has an average diameter of about 500 micrometers and was wrapped with about a 1500 micrometer spacing. 16 gauge (approximately 0.16 cm diameter) wire composed of alloy A was then arc sprayed onto the Nicalon fiber wrapped mandrels for approximately 2.5 min. Arc spraying was performed at approximately 34 volts, 100 amps to deposit the required layer of rapidly solidified alloy A. FIG. 2 is a light photomicrograph of fiber reinforced arc sprayed monotape composed of rapidly solidified aluminum base alloy A deposited on reinforced Nicalon placed upon planar flow cast aluminum based alloy A ribbon fabricated by the present invention. Some porosity may be observed due to the fact that arc spraying is not done in vacuum, however, discrete primary intermetallic

compound particles are not seen in the matrix alloy A microstructure indicating that solidification of the arc sprayed metal droplets occurs at a rate rapid enough to suppress the formation of coarse primary dispersoid particles.

### EXAMPLE III

Transmission electron microscopy (TEM) was performed on arc sprayed monotape to further examine the microstructure of the deposited layer. Samples were 10 prepared by mechanically grinding off the planar flow cast alloy A substrate and thinning the sample to approximately 25 microns in thickness. TEM foils were prepared by conventional electro-polishing techniques in an electrolyte consisting of 80 percent by volume 15 methanol and 20 percent by volume nitric acid. Polished TEM foils were examined in an Philips EM Philips 400T electron microscope. Transmission electron photomicrographs of a deposited layer of arc sprayed alloy composed of rapidly solidified aluminum based 20 iron, vanadium and silicon containing alloy fabricated by the present invention is shown in FIG. 3.

### EXAMPLE IV

Arc sprayed monotapes of BP fiber reinforced com- 25 posites were diffusion bonded for preliminary mechanical property screening. Two layers of rapidly solidified, planar flow cast aluminum based 2.37 at % iron, 0.27 at % vanadium and 1.05 at % silicon containing alloy ribbon approximately five centimeters by ten centimeters in dimension; were placed in between six layers of BP fiber reinforced plasma sprayed monotapes of approximately the same size as fabricated by the conditions prescribed to in Example I. Diffusion bonding was performed for a period of 1 hr. in a 445 kN vacuum hot press, at a temperature of approximately 500° C., under a pressure of approximately 50 MN/m<sup>2</sup>, and in a vacuum less than 10 microns of mercury. Photomicrographs of diffusion bonded layers of arc sprayed monotapes composed of rapidly solidified aluminum base 40 alloy A deposited on reinforced BP fiber placed upon planar flow cast aluminum base alloy A containing ribbon fabricated by the present invention showed good bonding.

### EXAMPLE V

Arc sprayed monotapes of Nicalon fiber reinforced composites were diffusion bonded for preliminary mechanical property screening. Six layers of rapidly solidified, planar flow cast aluminum based 2.37 at % iron, 0.27 at % vanadium and 1.05 at % silicon containing alloy ribbon, approximately five centimeters by ten centimeters in dimension, were placed in between two layers of Nicalon fiber reinforced arc sprayed monotapes of approximately the same size as fabricated by the 55 conditions prescribed to in Example III. Diffusion bonding was performed for a period of 1 hr. in a 445 kN vacuum hot press, at a temperature of approximately 500° C., under a pressure of approximately 50 MN/m<sup>2</sup>, and in a vacuum less than 10 microns of mercury. Photomicrographs of diffusion bonded layers of arc sprayed monotapes composed of rapidly solidified aluminum base alloy A deposited on reinforced Nicalon fiber placed upon planar flow cast aluminum base alloy A containing ribbon fabricated by the present invention 60 showed good bonding.

Having thus described the invention in rather full detail, it will be understood that such detail need not be

strictly adhered to by that further changes and modifications may suggest themselves to one skilled in the art, all falling within the scope of the invention as defined by the subjoined claims.

We claim:

1. A process for producing a rapidly solidified aluminum base metal matrix composite, comprising the steps of:
  - (a) forming a rapidly solidified aluminum base alloy into a wire;
  - (b) arc spraying said wire onto at least one substrate having thereon a fiber reinforcing material to form a plurality of preforms wherein each of said preforms has a layer of said alloy deposited thereon and said fiber reinforcing material is present in an amount ranging from about 0.1 to 75 percent by volume thereof; and
  - (c) bonding said preforms to form an engineering shape.
2. A process as recited in claim 1, wherein said rapidly solidified alloy has a substantially uniform structure.
3. A process as recited in claim 2, wherein said rapidly solidified aluminum base alloy is prepared by a process comprising the steps of forming a melt of the aluminum based alloy and quenching the melt on a moving chill surface at a rate of at least 10<sup>5</sup>° C./sec.
4. A process as recited in claim 1, wherein said alloy layer is strongly bonded to said fiber reinforcing material.
5. A process as recited by claim 1, wherein in sequence, prior to step (c), additional fiber reinforcing material is applied to each of said preforms and said wire is arc sprayed thereon to modify said preforms prior to bonding.
6. A process as recited by claim 5, wherein said sequence is repeated a plurality of times.
7. A process as recited by claim 6, wherein said sequence is repeated from 2 to 10 times.
8. A process as recited by claim 5, wherein said modified preforms are bonded to form said engineering shape.
9. A process as recited by claim 5, wherein at least one of said modified preforms is bonded to at least one of said preforms to form said engineering shape.
10. A process as recited in claim 1, wherein said bonding step is at least one member selected from the group consisting of diffusion bonding, roll bonding and hot isostatic pressing.
11. A process as recited in claim 3, wherein said rapidly solidified aluminum based alloy has a composition consisting essentially of the formula  $Al_{a+b}Fe_aSi_bX_c$  wherein X is at least one element selected from the group consisting of Mn, V, Cr, Mo, W, Nb, Ta, "a" ranges from 1.5 to 8.5 at %, "b" ranges from 0.25 to 5.5 at %, "c" ranges from 0.05 to 4.25 at % and the balance is aluminum plus incidental impurities, with the proviso that the ratio [Fe+X]:Si ranges from about 2.0:1 to 5.0:1.
12. A process as recited in claim 11, wherein said rapidly solidified aluminum based alloy is selected from the group consisting of the elements Al-Fe-V-Si, wherein the iron ranges from about 1.5-8.5 at %, vanadium ranges from about 0.25-4.25 at %, and silicon ranges from about 0.5-5.5 at %.
13. A process as recited in claim 3, wherein said rapidly solidified aluminum based alloy has a composition consisting essentially of the formula  $Al_{a+b}Fe_aSi_bX_c$

wherein X is at least one element selected from the group consisting of Mn, V, Cr, Mo, W, Nb, Ta, "a" ranges from about 1.5-7.5 at %, "b" ranges from about 0.75-9.0 at %, "c" ranges from 0.25-4.5 at % and the balance is aluminum plus incidental impurities, with the proviso that the ratio [Fe+X]:Si ranges from about 2.01:1 to 1.0:1.

14. A process as recited in claim 3, wherein said rapidly solidified aluminum based alloy has a composition consisting essentially of the formula  $Al_{ba}Fe_aSi_bX_c$  10 wherein X is at least one element selected from the group consisting of Mn, V, Cr, Mo, W, Nb, Ta, Ce, Ni, Zr, Hf, Ti, Sc, "a" ranges from about 1.5-8.5 at %, "b" ranges from about 0.25-7.0 at %, and the balance is aluminum plus incidental impurities.

15. A process as recited in claim 3, wherein said rapidly solidified aluminum based alloy has a composition consisting essentially of about 2-15 at % from a group consisting of zirconium, hafnium, titanium, vanadium, niobium, tantalum, erbium, about 0-5 at % calcium, 20 about 0-5 at % germanium, about 0-2 at % boron, the balance being aluminum plus incidental impurities.

16. A process as recited in claim 3, wherein said rapidly solidified aluminum based alloy has a composition consisting essentially of the formula  $Al_{ba}Zr_aLi_bMg_cTd$ , 25 wherein T is at least one element selected from the group consisting of Cu, Si, Sc, Ti, B, Hf, Cr, Mn, Fe, Co and Ni, "a" ranges from about 0.05-0.75 at %, "b" ranges from about 9.0-17.75 at %, "c" ranges from about 0.45-8.5 at % and "d" ranges from about 0.05-13 30

at %, the balance being aluminum plus incidental impurities.

17. A process as recited in claim 1, wherein said fiber reinforcing material comprises at least one member selected from the group consisting of carbides, borides, nitrides and oxides.

18. A process as recited in claim 17, wherein said fibers are selected from the group consisting of silicon carbide and aluminum oxide.

19. A process as recited in claim 1, wherein said arc spraying step comprises the steps of (i) striking an arc between two strands of said wire to melt the tips thereof; and (ii) atomizing said melt in said arc by impinging a high pressure inert gas thereagainst.

20. A process as recited in claim 19, wherein said wire can range in size from 0.25 cm to 0.5 cm in diameter.

21. A process as recited in claim 19, wherein said wire can range in size from 0.1 cm to 0.18 cm in diameter.

22. A process as recited in claim 10, wherein said bonding step is carried out at a temperature ranging from 400° C. to 575° C., under applied pressure ranging from 7 MPa to 150 MPa.

23. A process as recited in claim 22, wherein said bonding step is carried out under applied pressure ranging from 34 MPa to 100 MPa.

24. A process as recited in claim 1, wherein aluminum foil is placed between preforms prior to bonding.

25. A process as recited in claim 1, wherein aluminum powder is placed between preforms prior to bonding.

\* \* \* \* \*